

# UNITED STATES PATENT OFFICE.

GEORGES HEBERLEIN, OF WATTWIL, SWITZERLAND.

## PROCESS FOR THE PRODUCTION OF PATTERN EFFECTS UPON COTTON FABRICS.

1,144,655.

Specification of Letters Patent. Patented June 29, 1915.

No Drawing.

Application filed May 29, 1914. Serial No. 841,805.

*To all whom it may concern:*

Be it known that I, GEORGES HEBERLEIN, a citizen of the Swiss Republic, and resident of Wattwil, Canton of St. Gall, Switzerland, have invented a new Process for the Production of Pattern Effects Upon Cotton Fabrics, of which the following is a full, clear, and exact specification.

A method of producing pattern effects upon cotton fabrics is known wherein concentrated sulfuric acid of from 45° to 55° Bé., which, as is known, serves to impart a parchmentizing action upon cellulose, is printed upon the fabric, which, after this action has taken place for a few seconds, is washed with water, or in which a resist is printed upon the fabric, after which the latter is passed for a few seconds through sulfuric acid, and finally washed. By this means those parts where the sulfuric acid acts upon the fibers, that is to say, those parts at which the so-called parchmentizing process takes place, become finer, thinner, and more transparent, while those parts which have not been acted upon by the sulfuric acid or have been reserved stand out as a pattern by reason of their less transparent quality and their greater thickness relatively to the more transparent background. Now, it has been found that with this process more distinctive ornamental effects can be obtained, if in carrying it out mercerized cotton fabric or fabric made of mercerized cotton and sulfuric acid of above 50½° Bé. are made use of. These enhanced effects, which would not be anticipated, are to be explained by the fact that the chemical alteration which cotton undergoes on being mercerized makes it more adaptable to reaction, whereby a greater transparency is ob-

tained in those parts of the fabric treated with sulfuric acid above 50½° Bé. than with unmercerized cotton. It is a curious fact that in the treatment of mercerized cotton fabrics with sulfuric acid a parchmentizing action only results when the concentration of the acid is in excess of 50½° Bé.

An extremely marked transparent effect is obtained in carrying out the process by allowing sulfuric acid of 54° Bé. to act upon the cotton fabric for about five seconds.

As the parchmentizing parts of the mercerized cotton fabric possess an exceedingly great affinity for several dye-stuffs, and on dyeing color much darker than the remaining portions of the fabric, the effect of the process is considerably heightened by the subsequent dyeing of the fabric.

What I claim is:

1. The described process for obtaining pattern effects upon cotton fabrics consisting of taking mercerized fabrics, subjecting the parts where pattern effects are to be produced for a few seconds to the action of sulfuric acid of over 50½° Bé. and finally washing out the acid.

2. The described process for obtaining pattern effects upon cotton fabrics consisting of taking mercerized fabrics, printing the required pattern on the said mercerized cotton fabrics with sulfuric acid of over 50½° Bé. and finally washing out the acid after a few seconds.

In witness whereof I have hereunto signed my name this 16th day of May, 1914, in the presence of two subscribing witnesses.

GEORGES HEBERLEIN.

Witnesses:

E. T. HÖRLER,  
C. MUHR.